

## UNITED STATES PATENT OFFICE

2,205,990

## PIPE THREAD LUBRICANT

Roy F. Nelson and William S. Hurwitz, Port Arthur, Tex., assignors to The Texas Company, New York, N. Y., a corporation of Delaware

No Drawing. Application January 15, 1938,  
Serial No. 185,157

9 Claims. (Cl. 87—9)

This invention relates to lubricating and coating compositions containing one or more metals in finely divided form. More particularly, the invention relates to compositions of matter which are useful for application to pipe threads and the like to prevent seizing, galling and stripping. Compositions which comprise a lubricating base composed of oil and a metal soap, and a soft metal in powdered form, such as commercial powdered zinc or lead, are typical.

In the construction of pipe lines, in the oil and natural gas industries, for example, a large number of relatively difficult problems have been encountered. One such problem which has caused considerable difficulty is encountered especially in the uncoupling of large sized threaded pipe joints. Such joints, after having been united for a short time, tend to "freeze" or grip tightly, the threads seize and stripping usually results. It has been recognized for some time that a special type of lubricant is required for such threaded joints and a considerable number have been proposed in the art.

Most of the pipe thread lubricants heretofore proposed have included one or more powdered solids dispersed in various types of lubricating bases. In some of the compositions of this type, particularly those containing powdered zinc, it has been found that upon standing for a period of time gas bubbles appear in said compositions and there is a tendency for the compositions to foam and to expand. This is undesirable as it is necessary to allow space for expansion in the containers in which the compositions are handled and marketed. It is also necessary to provide openings in said containers for the escape of said gases. The quality and stability of such compositions may be affected adversely by the formation and escape of gases therefrom, and accordingly said compositions may be improved by preventing the formation of said gases.

The reason for the formation and escape of gases from such compositions is not definitely known. Some of the gases so produced have been collected, however, and found to contain substantial quantities of hydrogen and of air. It has also been found that powdered zinc reacts with a number of the constituents of such compositions to produce hydrogen. The following

combinations of materials, for example, were mixed with zinc dust:

|                                                        |    |
|--------------------------------------------------------|----|
| Petroleum lubricating oil and water                    |    |
| Petroleum lubricating oil, water and lime              | 5  |
| Petroleum lubricating oil, water and high acid tallow  |    |
| Petroleum lubricating oil and high acid tallow         |    |
| Petroleum lubricating oil and lime                     |    |
| High acid tallow                                       | 10 |
| High acid tallow and water                             |    |
| Petroleum lubricating oil, aluminum sulfate and water  |    |
| Petroleum lubricating oil and aluminum sulfate         |    |
| Petroleum lubricating oil, aluminum stearate and water | 15 |
| Petroleum lubricating oil and aluminum stearate        |    |
| Petroleum lubricating oil, stearic acid and water      |    |
| Petroleum lubricating oil and stearic acid             |    |
| Petroleum lubricating oil, sodium sulfate and water    | 20 |
| Petroleum lubricating oil and sodium sulfate           |    |
| Stearic acid and water                                 |    |
| Stearic acid                                           |    |

In each case there was evidence of some type of reaction occurring in these mixtures within 48 hours of the mixing. In the case of the fluid mixtures, evolution of gas was noted by the bubbles developed in the liquid. In the mixtures containing fat, which were solid, evidence of reaction was noted by the swelling of the mixtures and apparent formation of gas pockets which may or may not have been hydrogen. It was observed that in mixtures of zinc dust and petroleum lubricating oil no gas was formed.

In the paint industry difficulty has been experienced in connection with the formation and escape of gases from coating compositions containing powdered zinc and drying oils such as linseed oil.

We have discovered that the formation and escape of gases from compositions of this type can be effectively prevented by introducing into the composition a small amount of nitrobenzene.

In a specific embodiment of our invention a pipe thread lubricant may be prepared, as follows:

A calcium soap grease of the type which is used in grease cups and the like may be prepared by saponifying tallow with lime, this

saponification being preferably conducted under steam pressure and in the presence of a small proportion of a petroleum lubricating oil. Upon release of the steam pressure an additional quantity of the petroleum lubricating oil may be worked into the mixture to produce a grease having the desired consistency. Finally zinc dust and a small amount of nitrobenzene may be mixed with the grease to produce a composition suitable for use as a pipe thread lubricant.

The pipe thread lubricant above described may contain, for example, the following ingredients, by weight:

|               | Per cent |
|---------------|----------|
| 15 Cup grease | 40 to 45 |
| Zinc dust     | 55 to 60 |
| Nitrobenzene  | 0.15     |

A cup grease may be used which has, for example, the following analysis:

|                                                    |                 |
|----------------------------------------------------|-----------------|
| Consistency, (A. S. T. M. method), unworked sample | 300-360         |
| Melting point                                      | 210° F. minimum |
| Calcium soap                                       | 10-14%          |
| 25 Free alkalinity, $\text{Ca}(\text{OH})_2$       | 0.2% maximum    |
| Foreign mineral matter                             | 0.1% maximum    |
| Free fatty acid, oleic                             | 0.2% maximum    |
| Free neutral fat (Sap. No. 196)                    | 2.0% maximum    |
| Water                                              | 2.0% maximum    |
| 30 Mineral oil                                     | 81.7% minimum   |

Zinc dust may be used which has, for example, the following analysis:

|                         |          |
|-------------------------|----------|
| Total zinc              | 97.2%    |
| 35 Metallic zinc        | 97.0%    |
| Zinc oxide              | 4.0%     |
| Iron and aluminum oxide | 1.6%     |
| Nickel                  | Negative |
| Copper                  | Negative |
| 40 Chromium             | Negative |
| Barium                  | Negative |
| Calcium                 | Negative |
| Lead                    | Negative |

The finished pipe thread lubricant may have, for example, the following specifications:

|                                                   |              |
|---------------------------------------------------|--------------|
| Consistency (A. S. T. M. method), unworked sample | 275-300      |
| Calcium soap                                      | 3-6%         |
| 50 Zinc dust                                      | 55-60%       |
| Water                                             | 1.0% maximum |
| Mineral oil                                       | 33% minimum  |

Other metal soaps may be used in preparing the lubricant base of these lubricants, including alkali metal, alkaline earth metal, and aluminum soaps.

It is possible to vary the proportions of the

various ingredients employed in our composition to a considerable extent. The amounts shown in the above examples are only illustrative. For example, the metal powder in the composition may range from about 10 per cent. to about 70 per cent. The proportion of petroleum lubricating oil may vary according to the consistency desired in the finished product. The amount of nitrobenzene which is required may vary, but ordinarily about 0.10% to 1.0% will be sufficient. 10

Obviously many modifications and variations of the invention, as hereinbefore set forth, may be made without departing from the spirit and scope thereof and only such limitations should be imposed as are indicated in the appended claims. 15

We claim:

1. A composition of the character described comprising an oil and powdered zinc which normally tends to deteriorate and form gas on standing, and a small amount of nitrobenzene 20 effective to stabilize said composition against such gas formation.

2. A pipe thread lubricant comprising a lubricating base such as a metal soap grease, a metal powder containing powdered zinc and a small amount of nitrobenzene. 25

3. A pipe thread lubricant comprising a calcium soap grease, a metal powder containing powdered zinc and a small amount of nitrobenzene.

4. A pipe thread lubricant comprising an aluminum soap grease, a metal powder containing powdered zinc and a small amount of nitrobenzene. 30

5. A pipe thread lubricant comprising from about 40% to about 45% of a calcium soap grease, 35 from about 55% to about 60% of powdered zinc and a small amount of nitrobenzene.

6. A pipe thread lubricant comprising from about 40% to about 45% of a calcium soap grease, from about 55% to about 60% of powdered zinc 4 and about 0.15% of nitrobenzene.

7. A pipe thread lubricant comprising from about 40% to about 45% of a calcium soap grease, from about 55% to about 60% of powdered zinc and from about 0.1% to about 1.0% of nitrobenzene. 4

8. A composition of the character described comprising a drying oil such as linseed oil, powdered zinc and a small amount of nitrobenzene.

9. In stabilizing a composition of the character described comprising an oil and powdered zinc, which tends to deteriorate and form gas on standing, the method which comprises adding thereto a small amount of nitrobenzene.

ROY F. NELSON.  
WILLIAM S. HURWITZ.